

K. SCHLECHT,  
PROCESS OF MAKING PRINTING BLOCKS,  
APPLICATION FILED NOV. 14, 1914.

1,412,093.

Patented Apr. 11, 1922.



INVENTOR

Karl Schlecht  
BY  
Mrs Wallace White  
ATTORNEY

# UNITED STATES PATENT OFFICE.

KARL SCHLECHT, OF BÖBLINGEN, GERMANY.

## PROCESS OF MAKING PRINTING BLOCKS.

1,412,093.

Specification of Letters Patent. Patented Apr. 11, 1922.

Application filed November 14, 1914. Serial No. 872,129.

(GRANTED UNDER THE PROVISIONS OF THE ACT OF MARCH 3, 1921, 41 STAT. L., 1313.)

*To all whom it may concern:*

Be it known that I, KARL SCHLECHT, a citizen of the German Empire, residing at Böblingen, in the Kingdom of Wurttemberg, Empire of Germany, have invented certain new and useful Improvements in Processes of Making Printing Blocks, of which the following is a specification.

This invention relates to the process of 10 making printing blocks by laying on the spots cleared by the development of a chromate colloid copy, a bed of resin or varnish capable of resisting the action of fats and acids, and has for its object the production 15 of a block having a uniform surface which will be more advantageous and economical for use in both direct and offset printing, and by means of which a large number of and particularly effective, impressions may 20 be obtained.

In the process of making printing blocks by laying on the spots cleared by the development of a chromate colloid copy, a bed of resin or varnish capable of resisting the 25 action of fats and acids, it has been found that the picture elements, consisting of a layer of resin or varnish, project a little higher than the remaining parts of the printing block. This is especially disadvantageous for offset printing because the 30 block wears unevenly, so that the number of clear impressions that can be obtained, is very limited, and the india rubber cloth of the offset press is worn out rapidly 35 by repeated contact with the uneven surface. The picture elements being exposed, they wear off very quickly and instead of producing a fine grain and clear impressions, a coarse grain and blurred impression 40 or picture, results.

My method of making these printing blocks is such that blocks are produced which have a substantially uniform printing surface, so that the number of impressions that may be obtained is greatly increased; and the india rubber cloth is not injured by the flat surface, so that wear is materially reduced.

I will describe one process embodying my 50 invention and will then point out the novel features thereof in claims:

The accompanying drawing illustrates somewhat diagrammatically, a preferred embodiment of my invention.

In the drawing, Fig. 1 is a fragmentary 55 sectional view showing a printing block or plate before etching and after the chromate colloid copy has been developed.

Fig. 2 is a view showing the plate after 60 etching.

Fig. 3 is a view showing the plate after coating with resin or varnish.

Fig. 4 is a view showing the plate after treating with turpentine.

Fig. 5 is a view showing the plate after 65 recoating with greasy ink alone.

Fig. 6 is a view showing the plate after treatment with nitric acid.

In all of the views, the sequence in which the ingredients are applied and removed 70 are indicated by the accompanying legends.

In carrying out the invention according to the drawing, the chromate colloid copy or layer K is first developed, and then rolled in with greasy ink H and dusted with asphalt powder A as shown in Fig. 1; is then warmed up and etched in diluted nitric acid or the like, so that the picture spots are reduced below the level of the rest of the plate B as shown in Fig. 2. The plate 80 B is now covered as shown in Fig. 3, with a solution of resin or varnish C which is insoluble in turpentine or benzine, and is then treated with turpentine or the like by means of which the greasy ink H and the covering 85 of asphalt powder A with the resin C adhering thereto is removed, leaving the picture spots or perspective plane still coated with the insoluble resin or varnish C as shown in Fig. 4. Due to the fact that 90 these picture spots are depressed below the rest of the plate B, the solution of resin penetrating into the spots is therefore laid on thicker than has hitherto been the case, so that these parts have a considerably increased power of resistance, when subsequently subjected to the graining and printing operation.

The graining is accomplished by rolling in the entire plate B once more with greasy 100 ink H as shown in Fig. 5 and then treating it with a solution of diluted nitric acid or the like, which removes the layer of colloid K and produces the graining upon the plate at the same time. By this operation the 105 surface of the plate B is reduced somewhat so as to correspond with the lower level of the picture spots. In this way, a flat

printing block is produced in which the design and the grain are substantially at the same level as shown in Fig. 6.

- This feature is of the greatest importance 5 for offset printing, as it enables a large number of clear impressions to be made, by preventing the sharp picture elements from being exposed and thus wearing off quickly, as distinct from the blurred and indistinct 10 impressions or pictures produced by coarse grain picture elements. Moreover, it is possible by varying the levels of the picture spots and the grained surface, to make a printing block that will, particularly in offset 15 printing, give very effective impressions. Furthermore, if it is desired the picture spots may be even depressed slightly below the grained surface of the block or plate, so that the ink collects on them in a 20 thicker layer; it is then raised by the india rubber cloth of the offset press and the laying on of the ink on the paper is more effective than can be obtained from blocks ordinarily in use. This method of making printing 25 blocks may of course be used for blocks intended for both offset printing and direct printing.

Having thus described my invention, what I claim and desire to secure by Letters-Pat- 30 ent is:

1. The method of making printing blocks from developed and etched chromate colloid plates from which the protecting colloid and resist have not been removed, which method 35 consists in coating the face of such plate with a resinous material so that the etched surfaces will become filled to the same plane as the original surface of the block and then removing the protecting colloid and its over- 40 lying resist and resinous coating.

2. The method of making printing blocks from developed and etched chromate colloid plates from which the protecting colloid and its overlying resist have not been removed, 45 the resist consisting of greasy ink and asphalt powder, which method consists in coating the entire surface of the plate with a solution of resinous material insoluble in turpentine, treating the plate with turpen- 50 tine to remove the greasy ink and asphalt powder and its overlying resinous material while leaving the etched portions coated

with resinous material, graining the plate by first rolling up with greasy ink and then subjecting it to the action of nitric acid to 55 remove the colloid layer and grain the un-etched surface of the plate while the etched portions are protected by the resinous material, whereby the grained surface and the etched surface will be reduced to substan- 60 tially the same level.

3. The method of making printing blocks from developed and etched chromate colloid plates from which the protecting colloid and resist have not been removed, which method 65 consists in coating the entire surface of the plates with a resinous material so that the etched surfaces will become filled to the same plane as the original surface of the block, removing the resist and resinous coating over- 70 lying the protecting colloid, and then subjecting them to the action of an acid to remove the colloid layer and grain the un-etched surface of the plates while the etched portions are protected by the resinous material, whereby the grained surface and the etched surface will be reduced to substan- 75 tially the same level.

4. The method of making printing blocks from developed and etched chromate colloid plates from which the protecting colloid and its overlying resist have not been removed, the resist consisting of greasy ink and asphalt powder, which method consists in coating the entire surface of the plates with 80 a solution of resinous material insoluble in turpentine, treating the plates with turpen- 85 tine to remove the resist and its overlying resinous material while leaving the etched portions coated with resinous material, and then subjecting them to the action of an acid 90 to remove the colloid layer and grain the un-etched surface of the plates while the etched portions are protected by the resinous material, whereby the grained surface and the etched surface will be reduced to substan- 95 tially the same level.

In testimony whereof I affix my signature in presence of two witnesses.

KARL SCHLECHT.

Witnesses:

RUDOLF WOLTERS,  
FRIDA KLAIBER.